

Sept. 2, 1952

P. MODIGLIANI

2,609,320

METHOD OF MAKING FLEXIBLE UNWOVEN FABRIC

Original Filed May 29, 1947

2 SHEETS—SHEET 1



INVENTOR.  
PIERO MODIGLIANI  
BY *Virgil C. Kline*

Sept. 2, 1952

P. MODIGLIANI

2,609,320

METHOD OF MAKING FLEXIBLE UNWOVEN FABRIC

Original Filed May 29, 1947

2 SHEETS—SHEET 2



INVENTOR.  
PIERO MODIGLIANI

BY *Virgil P. Kline*

## UNITED STATES PATENT OFFICE

2,609,320

## METHOD OF MAKING FLEXIBLE UNWOVEN FABRIC

Piero Modigliani, Manhasset, N. Y., assignor to  
 Johns-Manville Corporation, New York, N. Y.,  
 a corporation of New York

Original application May 29, 1947, Serial No.  
 751,481. Divided and this application December  
 9, 1950, Serial No. 200,020

11 Claims. (Cl. 154—90)

1

The instant invention relates to improved methods of making unwoven fabrics of thermoplastic filaments, such as glass, and is a division of my copending application, S. N. 751,481, filed May 29, 1947, in which the products of the instant method are claimed.

Heretofore, filamentary mats of glass have been formed in various ways. In one method glass fibers are drawn directly from a melting furnace or furnaces and accumulated on a rotating drum. The furnace and drum are relatively reciprocated so that the filaments of each of the layers accumulated on the drum are crossed with respect to the filaments of adjacent layers. In the normal practice the reciprocation is relatively slow as compared to the rate of fiber drawing, whereby the angles between the filament of adjacent layers are acute. When the mat is built up to the desired thickness it is removed from the drum by slitting its longitudinally of the drum, and the mat is then stretched in a direction substantially perpendicular to the original lay of the filaments, whereby it is expanded or opened in a manner similar to that of a "lazy tongs," the angles between the filaments opening to increase the porosity and to reduce the density and thickness of the product. The relatively loose, weak, fibrous product thus formed has, for a number of uses, been impregnated with a suitable binder to strengthen it and give it sheet-like characteristics. The impregnation of the product, however, binds the filaments relatively rigidly in their positions and greatly reduces the flexibility of the product. The principal object of the instant invention is the provision of methods of making unwoven fabric or sheets composed of glass filaments which will have the ability to readily flex and conform to irregular surfaces. More particularly an object of the invention is the provision of a method in which a minor proportion of an uncured adhesive or binder is distributed in an unexpanded mat of the type made on the drawing drum of the known equipment described above, the binder being applied during the drawing operation or after the mat is removed from the drum, but preferably the former. The mat is treated to soften the binder and urge it toward the crossing points of the filaments and is then expanded to a predetermined degree and in a direction at substantially right angles to the original lay of the filaments, and the binder is set or cured. The expansion step may be carried out in different ways and to different extents depending upon the characteristics desired for the finished product. However, in all

2

cases the operations are such that the fibers are reoriented and the product, as compared to the original mat, is relatively soft, thick and open.

5 My invention will be more fully understood and further objects and advantages will become apparent when reference is made to the more detailed description of a preferred embodiment of the invention which is to follow and to the accompanying drawings in which:

Fig. 1 is a perspective view of a product made in accordance with the method of the instant invention;

15 Fig. 2 is a view similar to Fig. 1 illustrating another product made by the method of the instant invention;

Fig. 3 is a diagrammatic, end elevational view of an apparatus employed in the instant invention for carrying out the method thereof;

20 Fig. 4 is a front elevational view of the apparatus of Fig. 3;

Fig. 5 is a diagrammatic, plan view of further apparatus employed in the instant invention particularly for the production of the product of Fig. 2;

25 Fig. 6 is a side, elevational view of the apparatus of Fig. 5;

Fig. 7 is a view similar to Fig. 5 illustrating apparatus employed to produce the product of Fig. 1; and

30 Fig. 8 is a side elevational view of the apparatus of Fig. 7.

Referring now to the drawings and particularly to Fig. 1, one product made by the method of the instant invention consists of an unwoven fabric 10 composed of a plurality of layers 12, each formed of continuous, or substantially continuous filaments 14. Fine glass filaments are preferably employed and the following description is directed particularly to such case. The filaments of each layer lie in approximate parallelism and, in this embodiment of the product, the filaments of adjacent layers cross each other at relatively acute angles; that is, the filaments lie generally longitudinally of the product, but at a sufficient angle to the longitudinal to cross the fibers of the adjacent layers. Intermingled with the filaments is a relatively minor proportion of a cured or hardened binder, the proportion of the binder being, say, 0.2 to 20% by weight of the product. The binder, illustrated at 16, exerts its binding action for the most part only at the intersection or crossing points of the filaments to bind the filaments firmly together at 45 these points. It will be understood that Fig. 1

55

is a diagrammatic illustration of the product and that in actual practice the binder will be visually relatively insignificant.

A glass fabric having the construction features described above is readily flexible and distortable due to the inherent flexibility of the individual filaments and the concentration of the binding action at the crossing points whereby the filaments may bend and distort intermediate such points. The product can readily be applied to irregular surfaces. It is very porous, open, and expanded or puffed up in thickness, and is adapted to absorb large percentages of impregnants. It can be used in many places in substitution for woven fabrics and in such uses has the further advantage that it contains none of the lubricants or sizings required for weaving operations.

The product may also be of a character to be highly stretchable and elastic, a product of this type being illustrated in Fig. 2. Fundamentally the product is similar to that in Fig. 1, except that the filaments lie at greater angles to the longitudinal dimension and, hence, cross each other at wider angles than before. The binder 16 exerts its binding function at the crossing points of the filaments, as in the case of the fabric of Fig. 1. The product is open and porous and relatively inflated or puffed up in thickness. When a product of this type is subjected to a pulling stress, although the fibers are firmly secured together at their crossing points, stretching will take place, due to the bending of the individual filaments, the filaments retaining their fixed relative positions in the fabric. When the pulling stress is released, the resilient characteristic of the fine glass rods which constitute the filaments, will urge them to again straighten out and return the fabric to substantially its original dimensions.

The binder employed for the products of both types may be either a thermo-setting or thermoplastic adhesive composition. The preferred material is an acrylic resin. Other binders, such as phenol-formaldehyde resins, urea-formaldehyde resins, polyvinyl alcohols, latex and the like may be used.

Referring now particularly to Figs. 3-8 inclusive, the method of making the products described above will be explained in detail. The initial mat, known as the "condensed" mat, is made by substantially the conventional drawing process previously described. Figs. 3 and 4 diagrammatically illustrate the essential steps in the formation of the initial mat and the apparatus employed therein. Fine glass filaments 22 in suitable number and integrally connected to glass issuing through the spinning orifices of a glass furnace 24, are brought into contact with a drawing drum 20, rotated in the direction indicated by the arrow in Fig. 3 by any suitable driving means and at relatively high speed, and continuously drawn directly from the glass furnace and accumulated on the drum. Furnace 24 is reciprocated relatively to the drum as indicated by the double-headed arrow in Fig. 4, to lay the glass filaments on the drum in a plurality of layers of continuous spirals with the filaments of each layer crossing the filaments of adjacent layers. The rate of reciprocation of the furnace relatively to the drawing speed, that is, the rotational speed of the drum, is such that the filaments of the adjacent layers cross each other at acute angles.

The binder application is preferably performed at suitable intervals during the drawing operation by a spray device 26 (see Fig. 3) which may

be a hand spray and which is moved back and forth across the mat on the drum to uniformly apply the binder material. The amount of binder used is carefully controlled to provide a solids binder content in the finished mat of, say, 0.2 to 20% by weight of the mat. The binder is preferably applied in the form of an emulsion, a water-dispersion of the preferred acrylic resin being suitable. However, a solution of the binder in a solvent may be employed. Due to the relatively high speed of movement of the mat carried on the drum, and the temperatures prevalent during the filament drawing operation, the binder rapidly dries by evaporation of the water, or the solvent, as the case may be, so that upon completion of the drawing operation, the mat contains a substantially dry, but unset binder.

Alternatively to apply the binder during the mat drawing operation, it may be sprayed or brushed on the mat after removal of the mat from the drum, and the mat then permitted to air dry. A conventional wetting agent of any suitable type may be used to insure penetration of the binder.

When the condensed mat is completed it is placed on a conveyor 28 in such a manner that the direction of the filament is generally transverse of the conveyor, as illustrated in Fig. 5; that is, the dimension of the mat measured by the circumference of the drum extends transversely of the conveyor. While the mat is on conveyor 28 it is treated with a binder softener. In the case of a binder such as the preferred acrylic resin, the softener is water which, in effect, again places the finely divided binder in suspension. If binders are employed of a type which cannot be practically softened with water, an appropriate solvent is used. The softener is applied by brushing it onto the mat, suitably with a hand brush 32, the brush strokes being made transversely of the conveyor; that is, in substantially the direction of the filaments on the conveyor. This operation softens or liquifies the uncured binder and tends to concentrate the binder at the crossing of the filaments. In lieu of the brush application of the binder, it may be applied by spraying or by a brush roll, but the hand brushing operation is preferred as it aids in the concentration of the binder at the crossing points. In addition to the softener a part of the binder may be applied at this stage. Thus a suitable percentage, say up to 70% of the total binder, may be applied at this time, the added binder being the same as that already used or one of the other binders, for example, a urea-formaldehyde resin. This may be spread onto the mat similarly as the softener. When the binder has been wetted and additional binder applied if desired, as described above, the mat is stretched and the binder set.

The stretching operations employed for the flexible, and for the flexible and elastic products, are fundamentally the same, but for best results vary in details. The apparatus illustrated in Figs. 5 and 6 is particularly adapted for the production of fabrics of the type shown in Fig. 2. The apparatus consists of a roll 30 adapted to overlie the conveyor 28 and to be pressed toward the conveyor by suitable means (not shown) to confine the mat between it and the conveyor, the roll and conveyor constituting a feeding device. Spaced from conveyor 28 and roll 30 a relatively short distance, say a foot or less, is a drafting or drawing device 34 of a suitable type which may consist as shown of driven rolls 36-38 and an overlying roll 40 rest-

ing thereon. Beyond the drafting device is a winder 42 consisting of driven rolls 43 and a spindle 45 adapted to rest on rolls 43. Binder curing means suitably consisting of series or rows of infra-red ray lamps 44, are positioned to direct their rays against the expanded mat or web. A row of the lamps may be positioned ahead of the drafting device above the web while two rows may be used behind the drafting device, one directed against the upper surface and one against the lower surface of the web. As will be appreciated, other binder curing devices may be used. A table 46 may be located between the conveyor 28 and drafting device to aid particularly in the threading of the mat through the device. Conveyor 28, roll 30, rolls 36 and 38 of the drafting device and the driven rolls 43 of winder 42 are driven by motors or devices (not shown) of conventional type, the drive being such that the speeds of the different driven elements may be respectively varied to permit necessary adjustments in the operation.

In the operation of the apparatus described above, a mat on conveyor 28 is carried into position to be confined between the conveyor and roll 30 and the mat is fed forwardly at a controlled rate by the conveyor and roll. As illustrated, more than one mat may be placed on a conveyor 28 whereby a mat may be undergoing treatment with the binder softener while a previously treated mat is being subjected to the stretching operation. In starting up the operation, the mat, as it emerges from between roll 30 and conveyor 28, is taken manually and as soon as a sufficient length of mat has appeared, is manually stretched out into the form of an extended web and inserted beneath roll 40 of the stretching device and thence carried to take-up spindle 45 of take-up device 42 and fastened to the spindle. At the completion of these starting steps the machine is operated to continuously stretch the mat. For this purpose rolls 36 and 38 are driven at a speed relative to the delivery rate of roll 30 and conveyor 28 to secure the desired elongation of the mat. In the production of the stretchable, elastic, resilient mat for which this apparatus is particularly adapted, the relative speed is such that the mat is stretched to, say, two to thirty times its original length, the filaments in the stretched product being shifted from positions where they lie approximately transversely of the mat to positions at wider angles, say, at angles approaching 45° in the commercial form. During the stretching operation, the filaments shift and slide on one another and the angles therebetween open up as illustrated in Fig. 5 to the extent determined by the relative speeds of the drawing and feeding devices. Inasmuch as the binder is in a softened and unset condition at this stage, it does not prevent the opening and stretching operation. The series or rows of lamps between the feeding and stretching devices initiates the curing of the binder but does not carry it through to such an extent as to harden the binder before the stretching operation is completed. As the stretched product leaves the drafting or stretching device 34 it is subjected to the binder setting action of the rows of lamps above and below the web which completes the setting and curing of the binder and removes the water or solvent employed to soften it. The finished web is then wound on winder 42 from whence it may be removed and divided into sheets, strips, tapes or the like, of the desired

shapes and dimensions. Rolls 43 of the winder are preferably driven at a speed only slightly greater than that of the rolls of the drafting device to tension the web or fabric so that it will not unduly wrinkle during the winding operation.

Referring now to Figs. 7 and 8, an apparatus is illustrated which is adapted particularly for the production of the flexible product of Fig. 1. Conveyor 28 and roll 30 may be the same as used in the previous case. A stretching or drafting device 48 which may be identical with the drafting device 34 of Figs. 5 and 6 is located at a substantial distance from the conveyor, say, a distance of 6 to 10 feet or more. Although not essential, a tensioning device 49 of any suitable or conventional type is located between the drafting rolls and the feeding means. In the construction illustrated, the tensioning device consists of bars 50 mounted on a frame pivoted as at 52, the bars tending to rotate in a clockwise direction on their pivot under the influence of a weighted lever arm 54. Devices for setting or curing the binder, consisting preferably of series of infra-red ray lamps, are located as in the previous embodiment, one series being supported between the feeding and drafting device and a second and third series being supported between the drafting device and a take-up 58. The latter may be in all respects the same as the take-up devices used in the embodiment of Figs. 5 and 6.

In the operation of this form of the apparatus the mat, after the application of the binder softening medium, is fed through the feeding device as before, and the drafting device is driven at a speed relative to the speed of the delivery device so as to stretch the mat into a web in which the filaments extend generally lengthwise and at acute angles to one another. For example, in commercial operations the mat has been stretched to over thirty times its original length. The wide spacing of the delivery device from the stretching means provides sufficient time for the extensive movement of the filaments necessary to secure their desired reorientation. The tensioning device, although not essential, is employed to aid in controlling the tension in the mat to obtain the desired rearrangement of the filaments.

The product produced by the method of Figs. 7 and 8 is very flexible and distortable as the filaments are free to bend between the adhesively locked crossing points. However, due to the arrangement of the filaments substantially longitudinally of the product, the product is relatively unstretchable. The mat made by the method and apparatus of Figs. 5 and 6 on the other hand, is not only flexible and distortable but also is stretchable and elastic. The application of pulling stresses to this product will cause bending of the filaments between their crossing points and, hence, stretching of the product, but due to the natural resilience of the filaments, upon removal of the pulling stresses, the filaments will return to substantially their normal condition.

Having thus described my invention in rather full detail, it will be understood that these details need not be strictly adhered to but that various changes and modifications may suggest themselves to one skilled in the art, all falling within the scope of the invention as defined by the subjoined claims.

## What I claim is:

1. A method of forming an unwoven fabric comprising forming a condensed mat of a plurality of layers of filaments with the filaments extending generally transversely of the mat and with the filaments of adjacent layers crossing at acute angles, applying an unset binder to the mat, expanding the mat in a direction transversely of the general lay of the filaments to form an elongated web, and setting the binder.

2. A method of forming an unwoven fabric comprising forming a condensed mat of a plurality of layers of filaments with the filaments extending generally transversely of the mat and with the filaments of adjacent layers crossing at acute angles, applying an unset binder to the mat during its formation, expanding the mat in a direction transversely of the general lay of the filaments to form an elongated web, and setting the binder.

3. A method of forming an unwoven fabric comprising forming a condensed mat by winding a plurality of layers of filaments on a drum with the filaments of adjacent layers crossing at acute angles, applying an unset binder to the filaments on the drum periodically during winding, expanding the mat to form an elongated web, and setting the binder.

4. A method of forming an unwoven fabric comprising forming a condensed mat of a plurality of layers of filaments with the filaments extending generally transversely of the mat and with the filaments of adjacent layers crossing at acute angles, applying an unset binder to the mat periodically during its formation, expanding the mat in a direction transversely of the general lay of the filaments to form an elongated web, and setting the binder.

5. A method of forming an unwoven fabric comprising forming a condensed mat of a plurality of layers of filaments with the filaments extending generally transversely of the mat and with the filaments of adjacent layers crossing at acute angles, applying an unset binder to the mat, the weight of the unset binder so applied being a minor proportion of the weight of said fabric, expanding the mat in a direction at right angles to the general lay of the filaments to form an elongated web, and setting the binder.

6. A method of forming an unwoven fabric comprising forming a condensed mat of a plurality of layers of filaments with the filaments extending generally transversely of the mat and with the filaments of adjacent layers crossing at acute angles, applying an unset binder to the mat during its formation, the weight of the binder so sprayed being a minor proportion of the weight of said fabric, expanding the mat in a direction at right angles to the general lay of the filaments to form an elongated web, and setting the binder.

7. A method of forming an unwoven fabric comprising forming a condensed mat of a plurality of layers of filaments with the filaments extending generally transversely of the mat and with the filaments of adjacent layers crossing at acute angles, spraying an unset binder on the mat periodically during its formation, the weight

5 of the binder so sprayed being a minor proportion of the weight of said fabric, expanding the mat in a direction at right angles to the general lay of the filaments to form an elongated web, and setting the binder.

8. A method of forming an unwoven fabric comprising forming a condensed mat of a plurality of layers of filaments with the filaments extending generally transversely of the mat and with the filaments of adjacent layers crossing at acute angles, applying an unset binder to the mat, the weight of the binder so applied being a minor proportion of the weight of said fabric, applying an agent to said mat to soften the binder, expanding the mat in a direction at right angles to the general lay of the filaments to form an elongated web, and setting the binder.

9. A method of forming an unwoven fabric comprising forming a condensed mat of a plurality of layers of filaments with the filaments extending in one general direction and with the filaments of adjacent layers crossing at acute angles, said mat containing a distributed, dried but unset binder, the weight of said binder being a minor proportion of the weight of said fabric, brushing a binder softener onto said mat in a direction to urge the binder toward the crossing points of the filaments, expanding the mat in a direction at right angles to the general lay of the filaments to form an elongated web, and setting the binder.

10. A method of forming an unwoven fabric comprising forming a condensed mat of a plurality of layers of filaments with the filaments extending in one general direction and with the filaments of adjacent layers crossing at acute angles, said mat containing a distributed, dried but unset binder in proportions of approximately 0.2% to 20% by weight of the mat, brushing a binder softener onto said mat in a direction to urge the binder toward the crossing points of the filaments, expanding the mat in a direction at right angles to the general lay of the filaments to form an elongated web, and setting the binder.

11. A method of forming an unwoven fabric comprising forming a condensed mat of a plurality of layers of filaments with the filaments extending in one general direction and with the filaments of adjacent layers crossing at acute angles, applying a thermo-setting binder in aqueous suspension to said mat during its formation, brushing a binder softener onto said mat in a direction to urge the binder toward the crossing points of the filaments, expanding the mat in a direction at right angles to the general lay of the filaments to form an elongated web, and setting the binder.

PIERO MODIGLIANI

## REFERENCES CITED

The following references are of record in the file of this patent:

## UNITED STATES PATENTS

| Number    | Name         | Date          |
|-----------|--------------|---------------|
| 2,546,230 | Modigliani   | Mar. 27, 1951 |
| 2,578,534 | Giles et al. | Dec. 11, 1951 |